

## UNITED STATES PATENT OFFICE

2,427,280

## NICKEL ELECTROPLATING COMPOSITION

Raymond A. Hoffman, Euclid, Ohio, assignor to  
 E. I. du Pont de Nemours & Company, Wil-  
 mington, Del., a corporation of Delaware

No Drawing. Application February 11, 1941,  
 Serial No. 378,413

2 Claims. (Cl. 204—49)

1

This invention relates to nickel plating and is more particularly directed to nickel plating processes and compositions wherein there is used as an addition agent an aliphatic sulfonic acid having a cyclic substituent.

Nickel plating baths have heretofore been modified by the inclusion of sulfonic acids or sulfation products of various organic compounds. Nickel plating baths containing such addition agents are of improved character but much is still left to be desired. While the prior art addition agents have usually effected some improvement in the character of deposit the agents individually are not sufficient to produce commercially desirable deposits and they must be used with another and sometimes with even two or more supplemental addition agents. Sometimes the addition agents while improving nickel deposits with respect to one characteristic, say brightness, are actually deleterious as to other essential characteristics such as ductility and freedom from pits. Either alone or in combination with other addition agents these sulfation and sulfonation products have not been all that could be desired.

It is an object of the present invention to provide nickel plating compositions and processes of improved character. It is a further object of the present invention to provide nickel plating compositions and processes by means of which ductile nickel deposits may be obtained. It is a still further object to provide nickel plating compositions and processes by means of which there may be produced bright and ductile nickel deposits. It is a still further object to provide nickel plating compositions and processes which will provide a nickel deposit of good character over a wide range of current densities. It is a still further object to provide addition agents which will benefit the nickel plating compositions and processes and the nickel deposits obtainable therewith. It is a still further object to provide an addition agent particularly applicable for the improvement of nickel chloride plating compositions and processes and the deposits obtainable therewith. It is a still further object to provide addition agents which may advantageously be used in nickel plating compositions and processes as a sole addition agent or which may advantageously be used with other addition agents. Still further objects will become apparent hereinafter.

The foregoing and other objects of this invention are attained by using as an addition agent for nickel plating baths an aliphatic sul-

5 fonic acid having a cyclic substituent. By the use of these addition agents deposits of excellent character are produced. These deposits are ductile and bright. The addition agents do not promote pitting and they increase the range of current densities over which deposits of good character can be produced. Not only are the addition agents markedly beneficial when used alone, but they possess an unusual capability for being used in combination with other addition agents known to the art to produce joint effects greater than would be expected from a consideration of the attributes of the individual agents.

10 Aliphatic sulfonic acids having a cyclic substituent may have as a substituent on the aliphatic group any aromatic or cycloaliphatic radical may be carbocyclic or heterocyclic and the heterocyclic radical may have as the hetero-atom such elements as oxygen, sulfur, and nitrogen. More specifically, there may be mentioned 15 phenyl-substituted alkyl sulfonic acids, furyl-substituted alkyl sulfonic acids, cyclopentyl-substituted alkyl sulfonic acids, and naphthyl-substituted alkyl sulfonic acids. The aliphatic group 20 may contain one or more sulfonic acid groups and these may be located on the same or different carbon atoms. It is generally preferable for the aliphatic to be a hydrocarbon group and for the aromatic substituent to be a hydrocarbon group except for the hetero-atom if any. The addition agent should be at least slightly bath soluble.

25 As typical aliphatic sulfonic acids with a cyclic substituent the following are given:

35

1.



2-phenyl ethylene sulfonic acid

40

2.



2-hydroxy-2-phenyl ethane sulfonic acid

45

3.



2-phenyl ethane sulfonic acid

50

55

4.   
2-phenyl ethane-1,1-disulfonic acid
5.   
3-phenyl propylene-2-sulfonic acid
6.   
3-phenyl propionaldehyde-2-sulfonic acid
7.   
3-phenyl propionic acid-2-sulfonic acid
8.   
(1-methyl-1-sulfo)-3-ethylene-6-methoxybenzene
9.   
(1-methyl-1-sulfo)-3-ethylene-5,6-methylene-dioxybenzene
10.   
(1-methyl-1-sulfo)-3-ethylene-5-methoxy-6-hydroxy-benzene
11.   
2-furyl ethylene sulfonic acid
12.   
2-hydroxy-2-furyl ethylene sulfonic acid
13.   
2-furyl ethane sulfonic acid

14.   
2-furyl ethane-1,1-disulfonic acid
15.   
2-furyl propionaldehyde-1-sulfonic acid
16.   
2-furyl propionaldehyde-1-methyl-1-sulfonic acid
17.   
ethylene-3-cyclopentyl-1-sulfonic acid
18.   
propionaldehyde-3-cyclopentyl-1-sulfonic acid
19. 2-naphthylethylene sulfonic acid.
20. 1,2-diphenyl ethylene sulfonic acid.
- It will be understood that while reference is made herein to sulfonic acids this term as is customary in the art is used to refer to either the free acid or to a bath-soluble salt. It is immaterial for purposes of this invention whether the free sulfonic acids are used or whether they are used in the form of bath-soluble salts since in any case the actual compound contained in the bath will depend upon the alkalinity or acidity. This practice is particularly mentioned in the Lutz-Westbrook Patent 1,818,229 just before the claims.
- The amount of an aliphatic sulfonic acid having a cyclic substituent to use will depend upon the particular bath and upon the particular effect desired. In general, from about one to twenty grams per liter of such an addition agent may advantageously be used. The best results were obtained in a sulfate-nickel plating bath with about two to four grams per liter of an aliphatic sulfonic acid having a cyclic substituent while in a chloride-nickel bath five to seven grams per liter was optimum. It will be understood that in either case larger or smaller amounts may advantageously be used but the specific ranges mentioned, under the particular conditions of bath operation, led to deposits of desired ductility and brilliance.
- When the addition agents of the present invention are used in conjunction with another brightening agent the amount of addition agent is ordinarily reduced by at least fifty per cent and the brightness of deposit is usually increased over that obtained with either brightener alone. In any event the amount of addition agent to use in any particular instance can best be determined by taking a small quantity of the particular bath to be improved and trying various

## 5

small quantities of the addition agent until the desired results are obtained. The amount can easily be determined by a few simple tests with the standard test cells now in common use by electroplaters for this purpose.

The addition agents of the present invention may advantageously be used with any of the addition agents known to the art of which those heretofore listed as shown in the Lutz-Westbrook, Schlotter, Waite, Pine, Harshaw, and Flett patents are typical. The so-called metal brighteners such as zinc or cadmium may also be used if desired and it may sometimes be found desirable to use sulfated higher alcohols. The addition agents of this invention may be used to advantage with a benzaldehyde having an oxygen substituent on the benzene ring such as meta-sulfobenzaldehyde or orthosulfobenzaldehyde.

While certain nickel plating baths are shown herein, it will be understood that the addition agents of this invention may advantageously be used in any nickel plating bath. The baths shown in the previously mentioned patents to Lutz-Westbrook, Schlotter, Waite, Pine, Harshaw, and Flett as well as those of the Lind-Harshaw-Long Patents 2,198,267 and 2,198,268 may advantageously be used.

The addition agents of the present invention have particularly great merit in chloride-nickel plating baths of a type recently developed. Such chloride-nickel plating baths are illustrated hereinafter in the examples, see for instance Example II, and they are characterized by containing chloride anion and sulfate anion in the ratio of 5:1 to 20:1 on the basis of molecular equivalents. In other words, the ratio



should equal from about 5 to 20, a figure close to the latter being preferable.

Nickel plating compositions according to the present invention may be offered to the trade as mixtures including suitable nickel compounds and a suitable aliphatic sulfonic acid having a cyclic substituent, the proportions of materials being such as to give upon solution in water a proper proportion of bath constituent. The aliphatic sulfonic acid having a cyclic substituent may of course be present either as the sulfonic acid or as a bath-soluble salt such as a sodium, potassium, amine, or nickel salt. The compositions as sold may contain any further addition agent which it is desired to use and it may sometimes be found desirable to sell mixtures of addition agents for inclusion in baths already made up. It will be understood that the term "nickel plating composition" is used herein in the customary way to refer to a packaged dry mixture as offered to the trade, to a concentrated solution suitable upon dilution for use as a plating bath either with or without the addition of further materials, and to the baths themselves.

As aliphatic sulfonic acids having a cyclic substituent which have been tested in plating baths with particularly interesting results I may mention 2-phenyl ethylene sulfonic acid, 2-hydroxy-2-phenyl ethane sulfonic acid, 2-phenyl ethane sulfonic acid, 2-phenyl ethane-1,1-disulfonic acid, 3-phenyl propionaldehyde-2-sulfonic acid, 2-furyl propionaldehyde-1-sulfonic acid, and 2-furyl propionaldehyde-1-methyl-1-sulfonic acid. The practice of my invention may be better un-

## 6

derstood by reference to the following illustrative examples:

## Example I

5 A nickel plating bath according to the present invention was made up as follows:

|                                                        |                 |     |
|--------------------------------------------------------|-----------------|-----|
| Nickel sulfate (NiSO <sub>4</sub> ·7H <sub>2</sub> O)  | grams per liter | 350 |
| Nickel chloride (NiCl <sub>2</sub> ·6H <sub>2</sub> O) | do              | 15  |
| Boric acid                                             | do              | 35  |
| 2-phenyl ethylene sulfonic acid                        | do              | 3   |
| Temperature                                            | °C              | 50  |
| pH                                                     |                 | 3.8 |

15 This bath was employed at current densities ranging from five to eighty amperes per square foot and gave beautiful nickel deposits which were bright, lustrous, and ductile.

20 The aliphatic sulfonic acid having a cyclic substituent which was used as an addition agent according to this example was prepared by treating styrene with sulfamic acid to form the amine salt of the sulfonic acid. The addition agent was used as the salt. Addition agents other than the 2-phenyl ethylene sulfonic acid may also be prepared by a similar reaction using apiol, safrol, anethol, eugenol, vinyl naphthalene, or other organic compounds having an unsaturated structure in the side chain for reaction with sulfamic acid to form the corresponding unsaturated sulfonic acid.

## Example II

25 A preferred chloride-nickel plating bath of the invention was made up as follows:

|                                                        |                 |     |
|--------------------------------------------------------|-----------------|-----|
| Nickel chloride (NiCl <sub>2</sub> ·6H <sub>2</sub> O) | grams per liter | 250 |
| Nickel sulfate (NiSO <sub>4</sub> ·7H <sub>2</sub> O)  | do              | 15  |
| Boric acid (H <sub>3</sub> BO <sub>3</sub> )           | do              | 50  |
| 2-phenyl ethylene sulfonic acid                        | do              | 5   |
| Temperature                                            | °C              | 55  |
| pH                                                     |                 | 3.5 |

30 Bright nickel deposits of excellent character were obtained from the bath of this example.

## Example III

35 A plating bath according to the present invention was prepared using two addition agents as in the following:

|                                                        |                 |     |
|--------------------------------------------------------|-----------------|-----|
| Nickel sulfate (NiSO <sub>4</sub> ·7H <sub>2</sub> O)  | grams per liter | 350 |
| Nickel chloride (NiCl <sub>2</sub> ·6H <sub>2</sub> O) | do              | 15  |
| Boric acid (H <sub>3</sub> BO <sub>3</sub> )           | do              | 35  |
| 2-phenyl ethylene sulfonic acid                        | do              | 1½  |
| m-Sulfobenzaldehyde                                    | do              | 3   |
| Temperature                                            | °C              | 50  |
| pH                                                     |                 | 3.8 |

40 Excellent bright nickel deposits were obtained from this bath.

## Example IV

45 A chloride-nickel bath was made up with two addition agents as follows:

|                                                        |                 |     |
|--------------------------------------------------------|-----------------|-----|
| Nickel chloride (NiCl <sub>2</sub> ·6H <sub>2</sub> O) | grams per liter | 250 |
| Nickel sulfate (NiSO <sub>4</sub> ·7H <sub>2</sub> O)  | do              | 15  |
| Boric acid (H <sub>3</sub> BO <sub>3</sub> )           | do              | 50  |
| 2-phenyl ethylene sulfonic acid                        | do              | 2½  |
| m-Sulfobenzaldehyde                                    | do              | 2½  |
| Temperature                                            | °C              | 55  |
| pH                                                     |                 | 3.5 |

50 Brilliant nickel deposits of excellent character were obtained over a wide range of current densi-

ties, five to eighty-five amperes per square foot, using this bath.

*Example V*

A chloride-nickel plating bath of this invention was made up using a different aliphatic sulfonic acid having a cyclic substituent as follows:

Nickel chloride ( $\text{NiCl}_2 \cdot 6\text{H}_2\text{O}$ )

|                                                              |        |
|--------------------------------------------------------------|--------|
| grams per liter                                              | 250    |
| Nickel sulfate ( $\text{NiSO}_4 \cdot 7\text{H}_2\text{O}$ ) | do 15  |
| Boric acid ( $\text{H}_3\text{BO}_3$ )                       | do 50  |
| 2-furylpropionaldehyde-1-methyl-1-sulfonic acid              | do 4   |
| Temperature                                                  | °C 55  |
| pH                                                           | 3.2 15 |

Deposits from this bath were ductile, bright, and of very "fluid" character. Bright deposits were obtained from about five to sixty amperes per square foot.

*Example VI*

A sulfate-nickel bath of the invention was made up as follows:

Nickel sulfate ( $\text{NiSO}_4 \cdot 7\text{H}_2\text{O}$ )

|                                                               |                   |
|---------------------------------------------------------------|-------------------|
| grams per liter                                               | 350               |
| Nickel chloride ( $\text{NiCl}_2 \cdot 6\text{H}_2\text{O}$ ) | do 15             |
| Boric acid ( $\text{H}_3\text{BO}_3$ )                        | do 35             |
| 2-hydroxy-2-phenyl ethane sulfonic acid                       | grams per liter 3 |
| Temperature                                                   | °C 50             |
| pH                                                            | 3.4 30            |

Smooth, pit-free, ductile deposits were obtained.

*Example VII*

Still another sulfate-nickel bath illustrative of the invention was made up as follows:

Nickel sulfate ( $\text{NiSO}_4 \cdot 7\text{H}_2\text{O}$ )

|                                                               |       |
|---------------------------------------------------------------|-------|
| grams per liter                                               | 350   |
| Nickel chloride ( $\text{NiCl}_2 \cdot 6\text{H}_2\text{O}$ ) | do 15 |
| Boric acid ( $\text{H}_3\text{BO}_3$ )                        | do 35 |
| 2-phenyl ethane sulfonic acid                                 | do 2  |
| Temperature                                                   | °C 50 |
| pH                                                            | 3.5   |

Bright, ductile deposits were obtained over the entire plating range.

*Example VIII*

A still further sulfate-nickel bath of the present invention was made up as follows:

Nickel sulfate ( $\text{NiSO}_4 \cdot 7\text{H}_2\text{O}$ )

|                                                               |       |
|---------------------------------------------------------------|-------|
| grams per liter                                               | 350   |
| Nickel chloride ( $\text{NiCl}_2 \cdot 6\text{H}_2\text{O}$ ) | do 15 |
| Boric acid ( $\text{H}_3\text{BO}_3$ )                        | do 35 |
| 2-phenyl ethane-1,1-disulfonic acid                           | do 2  |
| Temperature                                                   | °C 50 |
| pH                                                            | 3.5   |

Bright, ductile deposits were obtained over the entire plating range.

*Example IX*

A still further sulfate-nickel bath illustrative of the present invention was made up as follows:

Nickel sulfate ( $\text{NiSO}_4 \cdot 7\text{H}_2\text{O}$ )

|                                                               |       |
|---------------------------------------------------------------|-------|
| grams per liter                                               | 350   |
| Nickel chloride ( $\text{NiCl}_2 \cdot 6\text{H}_2\text{O}$ ) | do 15 |
| Boric acid ( $\text{H}_3\text{BO}_3$ )                        | do 35 |

Bright, ductile deposits were obtained over the entire plating range.

3-phenylpropionaldehyde-2-sulfonic

|             |    |     |
|-------------|----|-----|
| acid        | do | 5   |
| Temperature | °C | 50  |
| pH          |    | 3.5 |

Bright, ductile deposits were obtained over the entire plating range.

*Example X*

A still further sulfate-nickel bath illustrative of the invention was made up as follows:

Nickel sulfate ( $\text{NiSO}_4 \cdot 7\text{H}_2\text{O}$ )

|                                                               |       |
|---------------------------------------------------------------|-------|
| grams per liter                                               | 350   |
| Nickel chloride ( $\text{NiCl}_2 \cdot 6\text{H}_2\text{O}$ ) | do 15 |
| Boric acid ( $\text{H}_3\text{BO}_3$ )                        | do 35 |
| 2-furylpropionaldehyde-1-sulfonic acid                        | do 5  |
| Temperature                                                   | °C 50 |
| pH                                                            | 3.5   |

Bright, ductile deposits were obtained over the entire plating range.

*Example XI*

A still further chloride-nickel bath illustrative of the invention was made up as follows:

Nickel chloride ( $\text{NiCl}_2 \cdot 6\text{H}_2\text{O}$ )

|                                                              |       |
|--------------------------------------------------------------|-------|
| grams per liter                                              | 250   |
| Nickel sulfate ( $\text{NiSO}_4 \cdot 7\text{H}_2\text{O}$ ) | do 15 |
| Boric acid ( $\text{H}_3\text{BO}_3$ )                       | do 50 |
| 2-furylpropionaldehyde-1-sulfonic acid                       | do 7  |
| pH                                                           | 3.5   |

Bright, ductile deposits were obtained over the entire plating range.

While I have shown illustrative aliphatic sulfonic acids having cyclic substituents in various illustrative baths and processes, it will be understood that without departing from the spirit of my invention one skilled in the art may readily devise numerous processes and compositions for nickel plating which are modified by the use of an aliphatic sulfonic acid having a cyclic substituent.

I claim:

1. A nickel plating composition for dissolving in water to make an aqueous plating bath comprising nickel chloride, nickel sulfate, and 2-phenyl ethylene sulfonic acid.

2. In a process for the deposition of nickel, the step comprising depositing nickel from an aqueous bath in the presence of 2-phenyl ethylene sulfonic acid.

RAYMOND A. HOFFMAN.

REFERENCES CITED

The following references are of record in the file of this patent:

UNITED STATES PATENTS

|           |             |               |
|-----------|-------------|---------------|
| Number    | Name        | Date          |
| 2,029,387 | Pine        | Feb. 4, 1936  |
| 2,312,097 | Hull et al. | Feb. 23, 1943 |

OTHER REFERENCES

Chemistry of Pulp and Paper Making—Sutermeister, 2d edition, (1929), published by John Wiley and Sons Inc., New York, page 182.

Wood Chemistry—Wise, published in 1944 by Reinhold Publishing Co., page 337.

**Certificate of Correction**

Patent No. 2,427,280.

September 9, 1947.

**RAYMOND A. HOFFMAN**

It is hereby certified that error appears in the printed specification of the above numbered patent requiring correction as follows: Column 2, line 17, after "radical" insert a period and words *The aromatic radical*; and that the said Letters Patent should be read with this correction therein that the same may conform to the record of the case in the Patent Office.

Signed and sealed this 25th day of November, A. D. 1947.

**[SEAL]**

**THOMAS F. MURPHY,**  
*Assistant Commissioner of Patents.*